

## UNITED STATES PATENT OFFICE

2,033,710

## COPPER ALLOYS

Franz R. Hensel, Indianapolis, Ind., and Earl I. Larsen, Newark, N. J., assignors to Westinghouse Electric & Manufacturing Company, East Pittsburgh, Pa., a corporation of Pennsylvania

No Drawing. Original application March 8, 1934, Serial No. 714,614. Divided and this application February 8, 1935, Serial No. 5,579

## 4 Claims. (Cl. 148—32)

This invention relates to alloys and particularly to copper base alloys which have improved mechanical, thermal and electrical properties.

Certain metals have been alloyed with copper to produce an alloy having better mechanical properties but generally such alloys have been quite inferior to copper as conductors of electricity and it has been difficult to duplicate the resulting characteristics.

10 An object of this invention is to produce an alloy of copper in which hardening elements are distributed throughout the resulting alloy in a finely divided state, improving the mechanical properties of the alloy and maintaining a 15 high electrical and thermal conductivity comparable to that of copper.

This application is a division of Serial No. 714,614, filed March 8, 1934, and directed to Copper alloys.

20 In order to produce a copper base alloy which will have desired mechanical and electrical properties, metals are added which can be precipitated to effect a dispersion of fine particles throughout a copper melt. It has been discovered that a copper alloy containing even small 25 proportions of chromium and cadmium has excellent mechanical and electrical properties when suitably heat treated.

The introduction of the chromium into molten 30 copper to form a solution is difficult, for chromium dissolves slowly in copper and the amount finally dissolved is small. The free chromium differs in density from copper and tends to segregate in the melt and to result in lack of homogeneity in the resulting solid product. Moreover, chromium being lighter than copper it is 35 difficult to keep the chromium submerged for the time required to dissolve it. The chromium tends to rise to the surface of the melt where 40 oxides are formed that contaminate the product.

In practice, finely divided chromium may be added to the copper melt in the form of a compacted mass or mixture in order that the chromium will be dissolved in and not tend to segregate from the copper melt. One of the preferred forms in which the chromium is added to the copper melt is as a cake, pellet or rod compacted from intermixed copper and chromium powders.

50 In producing the cake, pellet or rod of intermixed copper and chromium powders, the copper and chromium melts are powdered to approximately 100 mesh size and then thoroughly mixed and compressed to sufficient density to prevent floating of the chromium from molten

copper. A pressure of about 60,000 lbs. per sq. inch on the intermixed copper and chromium powders produces a mass which has a density of about 8.5. Lower pressures and densities, however, may be employed.

Another method of preparing the powdered copper and chromium metals in the form desired is to alternately compress the powdered mixture under a pressure of 4000 lbs. per sq. inch and then heat the compressed mass in a reducing atmosphere to sinter the particles. A modification of this method is to heat the compressed mass in a reducing atmosphere to approximately the melting point of copper and to quickly strike the mass a hard blow as in a die under a punch 15 press.

The finely divided chromium powder may also be enclosed in copper tubes of suitable size instead of in the form of compressed and sintered masses hereinbefore described. The copper 20 tubes which contain the chromium powder are swaged to suitable compactness for addition to the molten metal. Such articles may be employed as hardening and scavaging additions to other alloys.

Satisfactory copper chromium alloys containing up to 5% of cadmium have been produced which have high mechanical properties and good electrical conductivity. The cadmium may be added to the copper melt either in the 25 form of pure cadmium or it may be added in the form of a fine powder compressed with the finely divided chromium and copper powders into a compact mass or mixture such as the cake, pellet or rod hereinbefore described.

Generally, the alloying content of the alloys prepared in accordance with this invention comprises from .1% to 5% cadmium with about .1% to 5% chromium and the balance copper. The relative amounts of cadmium and chromium content in the copper base alloy is adjusted according to the hardness or strength and conductivity desired.

These copper base alloys have excellent mechanical and electrical properties and may be 45 employed in making sand castings of complicated design. In casting the alloys where the chromium content is above 1.5% there is a tendency for the chromium to separate and segregate and float to the top of the casting and to thus produce unsound castings. This segregational effect of the high chromium content in the alloy may be reduced by the use of rapidly cooled types of molds. Slower cooled types of molds may be employed where the chromium content of the alloy is about 50 55

.5%. The alloys formed by such an addition have good pouring qualities and when suitably heat treated have excellent mechanical and electrical properties.

5. In practice, the castings made from the copper base alloys are aged by suitable heat treatment to develop the mechanical and electrical properties of the alloy. A method which has been found to be satisfactory for developing the properties of the alloy is to heat the casting to between 600° C. and 1000° C., quench or quickly cool it and then reheat it to between 250° C. and 600° C. Where feasible, an intermediate cold working step may be interposed between the 10 quenching and ageing steps.

Alloys whose alloying contents are within the ranges hereinbefore described when heat treated in the above manner have excellent mechanical and electrical properties. An alloy comprising 15 cadmium as high as 2% with about 1% chromium and the balance copper when quenched from 950° C. had a hardness of 59 Brinell. After this alloy has been aged at 450° C., the alloy has a hardness of 116 Brinell. When quenched, the 20 alloy has a conductivity of only 50% of that of copper but after ageing, tests conducted show that the conductivity of the alloy has increased to 90% of that of copper.

Alloys prepared from these alloying elements 25 and within the ranges given above are particularly useful in the manufacture of large castings such as commutator segments and collector rings for dynamo electric machines, these alloys having high strength and high conductivity are particularly adapted to be employed as tips for mechanically operated welding electrodes, or as 30 welding wheels, or as current collecting nozzles

on automatic arc welding heads. Further, an important use for these high strength alloys is a cylinder head for internal combustion motors such as for automobile engines. These fields require a metal of high electrical and thermal conductivity combined with high strength at somewhat elevated temperatures. These alloys are found suitable for use at normal or low temperatures as required for transmission wires.

It is, of course, to be understood that various 5 modifications may be made in the alloying constituents and heat treatment as above described without in any way departing from the spirit of the invention, as set forth in the appended claims.

We claim as our invention:

1. An alloy comprising about .1% to 5% chromium, about .1% to 5% cadmium and the balance copper.

2. An alloy comprising 1% to chromium, 2% to cadmium and the balance copper.

3. An age hardened copper base alloy comprising from .1% to 5% chromium, from .1% to 5% cadmium with the balance copper which has been quenched from a temperature of between 600° C. and 1000° C. and reheated to and aged at a 25 temperature of between 250° C. and 600° C. to develop hardness and conductivity.

4. An age hardened copper base alloy comprising from .1% to 5% chromium, from .1% to 5% cadmium with the balance copper which has been 30 quenched from a temperature of between 600° C. and 1000° C., cold worked, and then reheated to and aged at a temperature of between 250° C. and 600° C. to develop hardness and conductivity.

35 FRANZ R. HENSEL.

EARL I. LARSEN.

#### CERTIFICATE OF CORRECTION.

Patent No. 2,033,710.

March 10, 1936.

FRANZ R. HENSEL, ET AL.

It is hereby certified that error appears in the printed specification of the above numbered patent requiring correction as follows: Page 2, second column, lines 19 and 20, claim 2, for "to" read of; and that the said Letters Patent should be read with these corrections therein that the same may conform to the record of the case in the Patent Office.

Signed and sealed this 26th day of January, A. D. 1937.

Henry Van Arsdale

Acting Commissioner of Patents.

(Seal)

.5%. The alloys formed by such an addition have good pouring qualities and when suitably heat treated have excellent mechanical and electrical properties.

5. In practice, the castings made from the copper base alloys are aged by suitable heat treatment to develop the mechanical and electrical properties of the alloy. A method which has been found to be satisfactory for developing the properties of the alloy is to heat the casting to between 600° C. and 1000° C., quench or quickly cool it and then reheat it to between 250° C. and 600° C. Where feasible, an intermediate cold working step may be interposed between the 10 quenching and ageing steps.

Alloys whose alloying contents are within the ranges hereinbefore described when heat treated in the above manner have excellent mechanical and electrical properties. An alloy comprising 15 cadmium as high as 2% with about 1% chromium and the balance copper when quenched from 950° C. had a hardness of 59 Brinell. After this alloy has been aged at 450° C., the alloy has a hardness of 116 Brinell. When quenched, the 20 alloy has a conductivity of only 50% of that of copper but after ageing, tests conducted show that the conductivity of the alloy has increased to 90% of that of copper.

Alloys prepared from these alloying elements 25 and within the ranges given above are particularly useful in the manufacture of large castings such as commutator segments and collector rings for dynamo electric machines, these alloys having high strength and high conductivity are particularly adapted to be employed as tips for mechanically operated welding electrodes, or as 30 welding wheels, or as current collecting nozzles

on automatic arc welding heads. Further, an important use for these high strength alloys is a cylinder head for internal combustion motors such as for automobile engines. These fields require a metal of high electrical and thermal conductivity combined with high strength at somewhat elevated temperatures. These alloys are found suitable for use at normal or low temperatures as required for transmission wires.

It is, of course, to be understood that various 5 modifications may be made in the alloying constituents and heat treatment as above described without in any way departing from the spirit of the invention, as set forth in the appended claims.

We claim as our invention:

1. An alloy comprising about .1% to 5% chromium, about .1% to 5% cadmium and the balance copper.

2. An alloy comprising 1% to chromium, 2% to cadmium and the balance copper.

3. An age hardened copper base alloy comprising from .1% to 5% chromium, from .1% to 5% cadmium with the balance copper which has been quenched from a temperature of between 600° C. and 1000° C. and reheated to and aged at a 25 temperature of between 250° C. and 600° C. to develop hardness and conductivity.

4. An age hardened copper base alloy comprising from .1% to 5% chromium, from .1% to 5% cadmium with the balance copper which has been 30 quenched from a temperature of between 600° C. and 1000° C., cold worked, and then reheated to and aged at a temperature of between 250° C. and 600° C. to develop hardness and conductivity.

35 FRANZ R. HENSEL.

EARL I. LARSEN.

#### CERTIFICATE OF CORRECTION.

Patent No. 2,033,710.

March 10, 1936.

FRANZ R. HENSEL, ET AL.

It is hereby certified that error appears in the printed specification of the above numbered patent requiring correction as follows: Page 2, second column, lines 19 and 20, claim 2, for "to" read of; and that the said Letters Patent should be read with these corrections therein that the same may conform to the record of the case in the Patent Office.

Signed and sealed this 26th day of January, A. D. 1937.

Henry Van Arsdale

Acting Commissioner of Patents.

(Seal)